

Patented Dec. 4, 1923.

1,475,942

# UNITED STATES PATENT OFFICE.

FRANK A. FAHRENWALD, OF CLEVELAND HEIGHTS, OHIO.

## ELECTRIC RESISTANCE ELEMENT.

No Drawing.

Application filed February 6, 1922. Serial No. 534,345.

To all whom it may concern:

Be it known that I, FRANK A. FAHRENWALD, a citizen of the United States, residing at Cleveland Heights, in the county of 5 Cuyahoga and State of Ohio, have invented a certain new and useful Improvement in Electric Resistance Elements, of which the following is a full, clear, and exact description, reference being had to the accompanying 10 drawings.

This invention relates to electrical resistance elements and has for its object the provision of a new alloy for the same which shall possess a high and uniform co-efficient 15 of resistance coupled with a high degree of resistivity to oxidation or other corrosive influences encountered in the use of such devices. Another object of the invention is the provision of an alloy which shall be 20 readily fabricated into the necessary physical forms, which shall possess a great rigidity of shape at high temperatures, which shall not become brittle, soft or "short" upon heating either continuously 25 or intermittently, which shall possess the same resistance at all times and which can be cheaply produced from materials of low intrinsic value; while further objects and advantages of the invention will become apparent as the description proceeds.

I employ iron as the base of my improved alloy because of its availability and cheapness; with it I alloy chromium for the purpose of increasing its melting point, and its 35 resistance to oxidation and other corrosion, and manganese for the purpose of overcoming its hardening or tempering qualities as well as increasing the specific electrical resistance. Carbon and silicon are present 40 as impurities but each to less than one-half of one percent, and preferably even less than that.

It is well known that electrical resistances are exposed to wide temperature variations, 45 in fact some times even being chilled or quenched as when a cooking element is splashed with water. If the element is made of an alloy which possesses hardening or tempering qualities, such as are characteristic of the steels, such treatment always tends to embrittle it and also causes resistance fluctuation; the resistance becomes suddenly increased upon such hardening, decreasing the temperature subsequently procurable with a fixed voltage until after a

sufficient length of time has elapsed for a complete annealing. In some cases the resistance is so much increased by the chilling that reheating of the element is very slow and the annealing likewise prolonged.

Of course it is the carbon present with the ferrous metal which produces this condition, and owing to the unavoidable presence of carbon as an impurity this condition is always present unless the peculiar hardening and tempering properties of the carbon be overcome by the addition of some other element of suitable nature and quantity. The range of choice is restricted by the considerations that the alloy must possess a high melting point, be non-corrodible, be malleable and ductile at all temperatures, stiff and strong at high temperatures, and possess a high and uniform co-efficient of electrical resistance. The only alloys which can fulfil these conditions are those which exhibit a solid solution condition throughout the entire range of working temperatures.

Chromium has the properties, when employed in sufficient quantity, of overcoming the hardening and tempering effect of carbon, but to produce this result by the addition of chromium alone requires upwards of twenty percent of chromium, indeed 80 twenty percent is hardly sufficient; but the addition of such a large amount of chromium gives rise to other grave difficulties, chief among which are the difficulty of fusing and working the bath, and the brittleness and lack of ductility of the alloy. The main reason for this condition is doubtless the presence of carbon as an impurity, since it is even more difficult to exclude carbon 85 from chromium alloys than from iron 90 alloys. It has been suggested to replace a portion of the chromium with nickel, since it is found that two parts of nickel has approximately the same effect in overcoming 95 the hardening effect of carbon as one part of chromium.

Nickel is further advantageous in possessing a higher resistance to oxidation than iron and a smaller affinity for carbon than either iron or chromium, and it produces 105 solid solution alloys of satisfactory physical properties when cold, although somewhat inclined to lop and sag when hot. The main drawback to the nickel alloy is its necessity of readjusting the proportion of chromium. 110

to iron at a ratio which is higher than that which occurs in nature.

It is also known that silicon, when alloyed with iron will overcome the hardening and tempering effects of carbon, but this property of silicon is not available for electrical resistance purposes owing to the fact that it renders the material "hot-short" when present in amounts greater than about 10 .5%. This is too small an amount to modify the carbon-quality perceptibly, since the effect of silicon is only about one fourth that of a like weight of chromium.

I have discovered that manganese can be 15 employed in connection with the chromium to overcome the carbon effect in producing quench-hardening of ferrous metal and with the production of an electrical resistance element possessing every one of the properties above enumerated as essential. It is true that manganese tends to lower the melting point and is, to this extent, a disadvantage, but its effect in overcoming quench-hardening is approximately twice that of 20 an equal weight of chromium, and its addition to iron, even in small quantities, has the result of considerably increasing the specific electric resistance. Accordingly I prefer to restrict the manganese to about 25 3% or less of the alloy. This enables me to decrease the chromium content to twenty per cent or less, thereby greatly facilitating the manufacture of the alloy, it enables the complete omission of nickel, which materially cheapens it, and it renders the alloy 30 more ductile at low temperatures and more rigid at high temperatures, without decreasing the melting point to such an extent as to interfere with the practical use of the alloy. 40 This quality, however, restricts the proportion which may be used.

I have had excellent results by the use of an alloy—

|             | Per cent.       |
|-------------|-----------------|
| 45 Chromium | 18              |
| Manganese   | 2 $\frac{1}{2}$ |
| Silicon     | .3              |
| Carbon      | .2              |
| Iron        | 79              |

50 The best range of my improved alloy for

electrical resistance purposes appears to be—

|              | Per cent. |
|--------------|-----------|
| Chromium     | 16 to 20  |
| Manganese    | 1 to 3    |
| Silicon      | .2 to .5  |
| Carbon       | .1 to .4  |
| Iron to make | 100       |

The foregoing can be considered either the furnace charge or the ultimate composition 60 of the alloy since if worked in a competent manner in an electric furnace the loss is negligible.

Ingots of such alloy can be forged into billets, rolled into rods, and drawn into wire 65 without cracks or seams. The first drawing can be effected hot, but after some working it can be drawn cold although the tensile strength is such as to render it desirable to elevate the temperature at all stages. Elements made therefrom can be heated even to 1800° F. and quenched without becoming hard or brittle or exhibiting any material change in resistance. The temperature coefficient is positive and low. The wire is 75 strong at all temperatures and even at 1800° F., does not sag when supported only at considerable intervals. It can be made from ordinary commercial ferrochrome and low carbon iron.

Having thus described my invention what I claim is:

1. An electrical resistance element made of an alloy of iron from about 16% to about 20% of chromium and about 1% to about 85 3% of manganese.

2. An electrical resistance element made of an alloy of iron with from about 16% to about 20% of chromium, and about 1% to about 3% of manganese, carbon and silicon being restricted to less than .5% each.

3. An electrical resistance element made of an alloy containing between about 16% to 20% of chromium and between about 1% and 3% of manganese, and the balance 95 mostly iron.

In testimony whereof, I hereunto affix my signature.

FRANK A. FAHRENWALD.